

1

2,911,415

## OPTICAL WHITENER

Harlan B. Freyermuth, Easton, Pa., and William W. Williams, New York, N.Y., assignors to General Aniline & Film Corporation, New York, N.Y., a corporation of Delaware

No Drawing. Application March 30, 1956  
Serial No. 574,999

3 Claims. (Cl. 260—329.3)

The invention here presented is a new whitener in the form of dye types of substances which are fluorescent under ultra violet or other light to yield a brilliant bluish white fluorescence; the agents being a series of 3,7-diaminodibenzothiophenedioxide sulfonic acids; particularly p-substituted amidobenzoyl derivatives.

It is well known that cellulosic materials such as paper, cotton textiles and the like have a slight yellowish hue which, particularly in the case of textile materials, is apt to become more pronounced when the material is subjected to repeated launderings and use. Accordingly, it has long been the practice to treat many white cotton textiles, when they are washed, with a bluing substance, such as ultramarine. It has been found that the slight blue coloration thus imparted to the material compensates for the yellowish tint or similar off-white shade of the material so that it appears whiter; such bluing operations, however, result in the absorption of a measurable portion of the total visible light falling upon the treated material and, accordingly, the treated material has a slightly dull appearance.

It has recently been proposed to treat paper or cotton textiles and similar cellulosic materials with agents which, while themselves colorless, fluoresce in the blue range



of the spectrum so that in daylight or other light, which includes ultra violet radiation, the fluorescence of the treating agent compensates for the slight yellowish tint or similar off-white shade, the blue being complementary to yellow. Such fluorescent agents only absorb a negligible portion of the visible light falling on the material and, accordingly, as a result of the fluorescence the treated material is much brighter as well as whiter in appearance.

While a wide variety of fluorescent agents have been suggested for treatment of fibrous materials, it has been found that for the treatment of cellulosic materials, either paper or textiles, the use of fluorescent agents which are substantive to cellulose is preferable since by the use of substantive fluorescent agents a whitening or brightening effect which is resistant to laundering is obtained.

Such substantive fluorescent agents have been applied to the material to be treated therewith either in a separate treating operation, or advantageously a small amount of the fluorescent agent may be incorporated in the soap or other detergent used for washing the textiles, and when the textile is washed with a detergent containing a fluorescent brightening agent, a small amount is picked up by the material so that after drying the material appears much whiter and brighter than untreated materials. These fluorescent brightening agents are also useful

2

in treating textile materials which are to be, or have been dyed or printed with discharge paste. The whites of the materials so printed with pastes containing brightening agents are much whiter than is otherwise the case.

While numerous fluorescent bleaching or brightening agents have heretofore been suggested, including diamino-stilbene sulfonic and carboxylic acids and certain acylated derivatives thereof, only a few of them have been satisfactory, particularly for use by incorporation in soap or other detergents. In order to be satisfactory for use as a brightening agent to be incorporated with soap or similar detergents, the fluorescent material which is employed should be itself colorless, or nearly so, and must not stain the material. It is necessary that it have a true bluish fluorescence with no tendency toward imparting visible yellow tints to the treated fabric. It must also have a proper degree of substantivity towards the materials as too small a degree of substantivity renders it valueless as it would be removed in any rinse waters, and too high a degree of substantivity results in a gradual build-up of fluorescent agent on material during repeated launderings resulting in off-color shades. The fluorescent agent must be stable to light and not discolor on exposure. It must also be stable to hypo-chlorite treatment and not discolor under such treatment, and, in addition, it must fluoresce over a fairly wide pH differential, including both alkali and acid.

The present invention presents a series of compounds which have some of the characteristics of dyestuffs or pigments, which in addition show a strong bluish white fluorescence of outstanding brilliance, which compounds in addition are readily incorporated into a wide range of fabrics, fibers, felted materials and paper, to yield an outstanding whiteness in the material to which they are applied. This material is a series of p-substituted amidobenzoyl derivatives which are best described as 3,7-diaminodibenzothiophenedioxide sulfonic acids. Broadly the compound has the following molecular structure:



where R may be lower alkyl, lower alkoxy, amino or lower mono or dialkylamino, y may be hydrogen or SO3z group; and z may be hydrogen, alkali metal ion or alkaline earth metal ion.

These compounds are readily prepared, for example, by condensing one molecular proportion of 3,7-bis(p-aminobenzoylamino)dibenzothiophene-dioxide-2,8-disulfonic acid with an excess of more than two molecular proportions of the appropriate amidating agent.

Examples of amidating agents are acetyl chloride, acetic anhydride, ethylchlorocarbonate (ethylchloroformate), dimethylcarbamyl chloride, methylisocyanate, etc.

3,7-bis-(p-aminobenzoylamino)dibenzothiophenedioxide-2,8-disulfonic acid is prepared by condensing one molecular proportion of 3,7-diaminodibenzothiophenedioxide-2,8-disulfonic acid with an excess of two molecular proportions of 4-nitrobenzoyl chloride and reducing the resultant dinitro derivative to the corresponding diamine.

These products are useful when incorporated into paper or other wrapping material to improve the whiteness as well as to protect the contents from the action of ultra violet light. When applied to textile fibers or fabrics by methods well known in the art, the whiteness is remarkably improved. The white background of photographic prints and diazotype prints can be improved by incorporating some of the material into the coating formula.

tions. By addition of the substances to discharge pastes, the whites obtained upon discharge are decidedly whiter than those discharges made in the absence of said materials. If small quantities of these materials are added to soaps or other detergents, fibers which are washed using these formulations will be much whiter in the case of whites and much brighter in the case of colors than fabrics which are washed with ordinary soaps or detergents. These materials may be used to bleach fabrics. In such cases, the amount of bleach necessary is materially reduced and one or more steps in the bleaching operation may be eliminated.



One of the more important properties of these compounds is their stability in the presence of sodium hypochlorite bleach materials together with their desirable shade of fluorescence; they are slightly bluer in shade of fluorescence than prior brighteners with the result that in daylight the whiteness of materials to which they are applied, is outstandingly enhanced. In addition they are free from any trace of green or pink tint in fluorescent properties.

Thus the product of the invention outstandingly increases the apparent whiteness of a wide range of materials by the incorporation thereinto of a dye type



substance of the triazinostilbene series containing 3,7-diaminodibenzothiophenedioxide sulfonic acid. Other objects and details of the invention will be apparent from the following description.

The following examples show the preferred method of practising the invention, but various modifications will be obvious to those skilled in the art.

The first step in the preparation of these substances consists in the production of necessary intermediates; as follows:

25.7 parts of 3,7-diaminodibenzothiophenedioxide-2,8-disulfonic acid and 176 parts pyridine were heated to 50° C. and 33 parts 4-nitrobenzoyl chloride was gradually added during two hours. 140 parts of a solution of 20% by volume sodium carbonate was added and the pyridine was removed by steam distillation. After all the pyridine was removed, the mixture was cooled to room temperature, filtered and the product dried in a vacuum oven at 65° C.

30 parts of the 3,7-bis(4-nitrobenzoyl) dibenzothiophenedioxide-2,8-disulfonic acid obtained from the preceding reaction was reduced with hydrogen in the presence of 5 parts Raney nickel catalyst employing 500 parts of water as the solvent. The reduction was carried out at 100° C. for six hours. Upon cooling, most of the Raney nickel catalyst was removed mechanically with a powerful magnet and the 3,7-bis(aminobenzoyl) dibenzothiophenedioxide-2,8-disulfonic acid was filtered and dried in a vacuum oven at 65-70° C.



With these two intermediates available, the new whitener may be prepared in its various embodiments as follows:

#### Example I

5 parts of 3,7-bis(aminobenzoyl)dibenzothiophenedioxide-2,8-disulfonic acid, 79 parts glacial acetic acid and 5 parts anhydrous sodium acetate were heated to reflux and 21.6 parts acetic anhydride was added gradually during 2 hours. After the acetylation was complete, the reaction mixture was poured onto 400 parts hot (70-80° C.) water to decompose the excess acetic anhydride. After one hour of stirring the product having the following structure was filtered and dried in a vacuum oven at 70° C.



#### Example II

10 parts of 3,7-bis(aminobenzoyl)dibenzothiophenedioxide-2,8-disulfonic acid and 98.2 parts pyridine were heated to 104° for five minutes in order to form the pyridine salt and then cooled to 10° C. 11.4 parts ethylchlorocarbonate were added during one-half hour. The reaction mixture was added to 1500 parts of water and the product isolated by the addition of 150 g. salt. The mixture was stirred for two hours and the product was then filtered and dried in the vacuum oven at 75° C. The product has the following structure:



When the substance of the present invention is applied to cotton from a warm soap solution, the cotton material shows an outstanding and valuable brightening and whitening effect.

When this material is incorporated into discharge pastes and applied to fabrics, the whites thus obtained were remarkably whiter than those obtained using ordinary discharge pastes. When this material is applied to fibers of cellulose, wool or nylon, by methods well known in the art, the white appearance of the fabric is thereby much improved.

If small amounts of this substance are added to soap or detergent and the resulting mixture is used to wash fabrics of cellulose, wool or nylon, the white materials thus washed are extraordinarily whiter in appearance and colored materials are brighter than similar materials which are washed using ordinary soaps or detergents.

The product and process of the invention thus provide material and procedures for outstandingly increasing the white appearance of a wide variety of surface substances. While there are above disclosed but a limited number of embodiments of the process of the invention it is possible to provide still other embodiments without departing from the inventive concept herein disclosed and it is therefore desired that only such limitations be imposed upon the appended claims as are stated therein or required by the prior art.

The invention claimed is:

1. A whitener having the formula



wherein R represents a member of the group consisting of lower alkyl and lower alkoxy and Z represents alkali metal.

## 2. A whitener having the formula



## 3. A whitener having the formula



## References Cited in the file of this patent

## UNITED STATES PATENTS

|           |                |       |                |
|-----------|----------------|-------|----------------|
| 2,529,860 | Amstutz        | ----- | Nov. 14, 1950  |
| 2,563,493 | Scalera et al. | ----- | Aug. 7, 1951   |
| 2,573,652 | Scalera et al. | ----- | Oct. 30, 1951  |
| 2,616,855 | Wheelock       | ----- | Nov. 4, 1952   |
| 2,624,710 | Thomas         | ----- | Jan. 6, 1953   |
| 2,635,969 | Goldstein      | ----- | Apr. 21, 1953  |
| 2,643,197 | Savidge et al. | ----- | June 23, 1953  |
| 2,649,385 | Kendall et al. | ----- | Aug. 18, 1953  |
| 2,702,759 | Scalera et al. | ----- | Feb. 22, 1955  |
| 2,706,178 | Young          | ----- | Apr. 12, 1955  |
| 2,719,155 | Siegrist       | ----- | Sept. 27, 1955 |
| 2,723,288 | Roberts        | ----- | Nov. 8, 1955   |
| 2,763,618 | Hendrix        | ----- | Sept. 18, 1956 |
| 2,765,239 | Siegrist       | ----- | Oct. 2, 1956   |